

## UNITED STATES PATENT OFFICE

ALBERT A. EPSTEIN, OF NEW YORK, N. Y., ASSIGNOR TO CONSOLIDATED PATENTEES CORPORATION, OF NEW YORK, N. Y., A CORPORATION OF NEW YORK

## COMBUSTIBLE PASTE

No Drawing.

Application filed November 13, 1930. Serial No. 495,538.

This invention relates to a combustible paste and also to a process for its production and has for its primary object the preparation of a paste having exceptional high burning characteristics and which may be effectively merchandised in collapsible containers or air proof wrappers.

An object of the invention is the preparation of a combustible substance which will burn over an extended period with a quiet, smokeless, non-sputtering flame.

Another object of the invention is the preparation of a combustible material which is non-explosive and incapable of spontaneous combustion and may be readily discharged from a container and burnt in this discharge position without possibility of igniting the material remaining within the container.

Another object of the invention is the production of a combustible paste that may be deposited in a burning position of any required volume and which will effectively produce the required volume of flame over an extended period without effecting the general formation of the paste during the burning process.

A feature of my invention resides in a method of producing a combustible paste by taking advantage of the insolubility of a combustible material when impregnated with a highly inflammable fluid such as alcohol.

Another feature of my invention resides in regulating the consistency of the combustible paste by varying the volume of alcohol with which a combustible substance is impregnated.

Besides the above my invention is distinguished in the combination of a combustible substance with an inflammable fluid, and an ingredient that will absolutely control the characteristics of the flame produced during the burning process.

With this and other objects in view the invention will be better understood from the following detailed description of one embodiment of my invention.

My invention is based upon the principle that alcohol (methyl, ethyl or denatured) forms a cream or paste with certain insoluble

stearate. The reaction involved is the partial solution of the magnesium stearate in alcohol, in consequence of which a material of pasty and cohesive consistency is obtained, embodying a high amount of a very combustible fluid (alcohol) which enables the paste to burn with a large volume of flame over an extended period. 55

Of course, it is to be understood that other combustible materials may be substituted for magnesium stearate such as various grades of fats, tallow and fatty acids to which is added a chemical to render the same practically insoluble. 60

With this material is mixed a highly inflammable fluid such as alcohol, as above set forth, the volume of alcohol in relation to the mass of the combustible material determining the consistency of the paste, thereby enabling the paste to be usable for a multiplicity of 65 purposes in the commercialization thereof. 70

## Example one

A suitable type of paste can be produced by mixing one part of a combustible material 75 (such as magnesium stearate) by weight, with two parts alcohol, by volume, stirring the mixture until a homogeneous mass is obtained.

## Example two

A suitable type of fat or fatty acid may be mixed with a metallic salt and a predetermined quantity of the mixture placed within a predetermined volume of alcohol and subject to agitation. 85

Due to the insolubility of the material and the chemical reaction between the salt and the fatty substance, the alcohol only partially dissolves the material, the remaining portion 90 of the alcohol being held in suspension by its mechanical mixture, with material.

For the purpose of modifying the character of the flame produced during the burning of the paste, various ingredients may be placed in the mixture each having an individual reaction upon the character and the color of the flame produced. As an example of such compounds, I cite the following examples: 95 100

*Example three*

To a predetermined quantity of combustible paste, produced as outlined above, I mix a small quantity of a soluble wood distillate, 5 such as turpentine.

*Example four*

To a suitable quantity of combustible paste, prepared as set forth above, I mix a predetermined portion of a soluble solid, such as 10 rosin or camphor.

*Example five*

To a predetermined quantity of the combustible paste, produced as above set forth, I add an insoluble solid such as finely powdered charcoal or other forms of carbon. 15

Of course, it is to be understood that various other ingredients may be added for modifying the character of the flame produced. 20 Due to the addition of the substances just set forth, the color of the flame ranges between blue and white, the alcohol in the compound cooperating in the production of a flame that 25 is smokeless. I have found from actual experience that the character and color of the residue, after a burning operation, may be controlled by the type of ingredient placed in the combustible paste outlined above. I 30 have also found from actual experience that when charcoal, lampblack or similar ingredients are added the combustion is considerably prolonged and a glowing residue of the carbonaceous material remains until the combustion 35 is complete.

In the production of the compound set forth in Example 3, I find excellent results can be accomplished by mixing 9 parts of 40 alcohol with one part of turpentine, stirring the solution until complete miscibility of the turpentine and alcohol is obtained. To this mixture, I add, during a constant stirring operation, 5 parts, by weight, of the combustible 45 material set forth above, such as magnesium stearate.

In carrying out my method for production of the compound set forth in Example 4, I take two parts of rosin or camphor and add 50 the same to 100 parts of alcohol to which turpentine has been added, then adding to this mixture 50 parts of a combustible material, as set forth above, subjecting the same to constant agitation.

In the production of the compound as set forth in Example 5, I take 100 parts of an alcohol-turpentine mixture, as produced in carrying out the method involved, in Example 3 and mix this with 17 parts of a combustible material, such as magnesium stearate. 55 To this is added 33 parts of finely powdered charcoal constantly agitating the mixture during the production of the compound.

Although I have only set forth a few of 65 the many types of products that may be pro-

duced, I wish it to be understood that many more can be produced in the use of my basic principles, one of the basic principles residing in the impregnating of a combustible material with alcohol to produce a paste that 70 may be directly burnt at the point of discharge and which will burn in a smokeless manner leaving a residue that may be readily removed from its supporting surface.

I also wish to state that I am of the opinion 75 that I am the first to impregnate a more or less insoluble combustible material, with an inflammable fluid, in the manner set forth above for the eradication of smoke during the burning of the combustible material. In 80 view of the many changes that may be involved in the carrying out of my basic principles I do not wish to be limited in protection in any manner, whatsoever, except as set forth in the following claims:

What I claim is:

1. A combustible paste comprising a mixture of one part of magnesium stearate by weight with two parts of alcohol by volume and a flame modifying ingredient added 90 thereto.

2. A combustible paste consisting of magnesium stearate, a volume of alcohol, a quantity of turpentine and finely powdered charcoal. 95

3. A combustible paste comprising 100 parts of a mixture of alcohol and turpentine, 17 parts of magnesium stearate and 33 parts of finely powdered charcoal.

In witness whereof I have hereunto set my 100 hand.

ALBERT A. EPSTEIN.

105

110

115

120

125

130